

Patented Mar. 5, 1929.

1,704,385

# UNITED STATES PATENT OFFICE.

ROBERT ABBOTT HADFIELD, OF WESTMINSTER, ENGLAND.

## MANUFACTURE OF STEEL PRODUCTS.

No Drawing. Application filed July 7, 1926, Serial No. 121,059, and in Great Britain April 29, 1926.

This invention has reference to the manufacture, in a regular and economical manner, of steel products sound in character as regards freedom from blow holes, rocks, pipes, 5 segregations or other like defects. As the invention is specially applicable to the production of rolled steel rails of a sound and reliable character, the manner of carrying it into effect will now be described with reference to such steel products without any intention however of limiting it to such rolled products.

In the manufacture of rolled steel rails, the usual procedure adopted is to produce a 15 heat of normally finished steel of the desired composition by some approved process in an open hearth furnace or other suitable furnace or apparatus, as for instance a Bessemer converter, to tap or deliver the heat of finished steel into a ladle, the composition of the steel being, if necessary, adjusted to suit requirement, either before or after tapping or delivering the steel into the ladle, to afterwards run off the molten steel from the ladle 20 into ingot moulds and afterwards to roll the ingots into rails of the desired weight and section. With this method of procedure, there is no certainty that the steel run off from the ladle into the ingot moulds 25 will produce sound steel ingots. In a large proportion of cases it will not. The ingots, on the contrary, are frequently of a porous or honeycomb nature, particularly towards their upper portions, due to gas evolved 30 from the steel during cooling, so that in order to obtain from such ingots a portion of steel approximately sound, a considerable percentage of the upper portion of the ingots has to be cut off and discarded. Often, 35 almost complete ingots have to be discarded, owing to their unsound condition. This adds considerably to the cost of manufacture. During cooling of a cast steel ingot, 40 piping thereof will, as well understood, also occur if the steel be of what is called a settling nature, due to the contraction of the steel from the central portion of the ingot in an outward direction consequent upon the chilling effect of the metal ingot mould used.

When a cast steel ingot pipes well, it is commonly considered that the steel of which it is formed is of sound quality. To determine, before casting, whether a heat of normally finished steel is of a good settling 45 nature, a sample of the steel is usually tested by casting it into a small metal mould by which it is quickly chilled, and if it settles well therein, that is to say, if a cavity is formed in the top of the small sample ingot thus formed, the heat of steel is regarded as 50 a good settling steel and therefore sound. The heat of steel is therefore cast into ingots which are afterwards rolled into rails. As a matter of fact however, although the steel may appear to be of a good settling 55 nature, it may nevertheless be and often is, of unsound nature. I have found that the chill test in a small metal mould is, to some extent, an illusive one, so far as determining the real soundness of the steel is concerned. 60 As a result, large quantities of rolled steel rails are made, and passed into railroad service, that are wholly unreliable and often cause serious railway accidents, as the statistics published from time to time by the 65 authorities concerned, amply prove.

The piping that occurs in steel ingots also assists in the production of faulty rails, because, although it is supposed that the pipe will be closed up and the metal around the 70 same caused to become welded up during the rolling of the ingots into rails, this will not actually take place, or not in an effective manner. In every case however a considerable proportion of the piped upper end of 75 the ingot has to be discarded before rolling the remainder into a rail. The formation of a pipe in an ingot of good settling steel can however be avoided by feeding molten metal to the top of the ingot, during the 80 cooling of the lower portion of the ingot. This can be done in various ways, as for example by the method and apparatus described in the specification of my former Letters Patent No. 933,731, No. 954,183, No. 95 85 1,172,279 and No. 1,301,072, according to which the ingot mould is formed with a head of refractory non-conducting material, for instance a sand head, which is charged with molten steel that is kept in a molten condition during cooling of the ingot, by heat produced by the combustion of fuel thereon, for a sufficient time to enable some of such 90 molten metal to descend and compensate for the contraction of the metal in the ingot 95 during the cooling thereof.

Now the present invention has for its object to enable rolled steel rails and other track structures, as well as other rolled or forged steel articles, as for instance, steel 100

105 110

plates and sheets, to be made with certainty, of steel of a thoroughly sound and reliable character throughout, in a regular and economical manner. It also has for its object 5 to enable not only steel made by the open hearth method but also steel made by the Bessemer method, which is now usually regarded as unsuitable for the manufacture of steel rails, to be used with confidence in 10 the manufacture of steel rails.

For this purpose, rolled steel rails and other rolled or forged steel articles, herein-after for brevity included in the term rolled steel rails, are made by producing a heat 15 of normally finished steel of the desired composition and of medium temperature, by any approved process, and then, before casting the steel into an ingot, testing a sample of the steel in a test mould formed of refractory material that will not rapidly chill the 20 test sample but will, on the contrary, allow it to cool only comparatively slowly, so that if the sample of steel contains such an amount of gas as would result in the production of 25 an unsound ingot, if the heat of steel were at once cast into an ingot, this fact would be indicated by the evolution of gas from the sample of steel in the mould causing the steel to rise, that is to say, to extend 30 more or less above the top of the mould. If, on the other hand, the sample of steel be of a sound and settling nature, a cavity will be formed in the top of the small ingot formed in the test mould, indicating that 35 the heat of steel is of a sound and settling nature and can therefore, without further treatment, be cast into an ingot from which a sound rail can be produced.

A mould of the character referred to, can 40 advantageously be formed of green sand. Such a mould may, for example be internally about six to eight inches in height and about one inch in diameter or width and be of cylindrical or prismatic shape. Or it 45 may internally be of an inverted conical or pyramidal shape so that it will be of gradually increasing cross-sectional area from bottom to top. Or a test mould of oblong shape and of about one and a half to two square 50 inches in section may be used. If the sample of steel tested in a mould of the kind referred to, rises, thus giving an indication that the steel is of an unsound nature, then there is thoroughly incorporated with the 55 heat of normally finished steel, whilst the same is in the furnace, or in a ladle into which it has been transferred, a sufficient quantity of a deoxidant, as for example aluminium or ferro-silicon, as will remove 60 the gas absorbed therein, or reduce it to so small a degree as to convert the steel into a sound and settling steel. This result may be ascertained by testing a sample of the treated steel in the same way as the un-

treated steel. The heat of treated steel, 65 when a sample thereof shows that it is of a settling nature, is then run off from the ladle into one or more ingot moulds provided with a refractory non-conducting head such as hereinbefore referred to. A test 70 mould made of dry sand has not so far been found satisfactory for the purpose mentioned.

During the cooling of the ingot, or each 75 ingot, molten steel is fed into the top of the ingot, in the way hereinbefore described, to prevent the formation of a pipe therein on cooling. In this way, an ingot of thoroughly sound and reliable steel can be produced. The ingot is afterwards rolled into 80 a rail of any desired weight and section which will be found to be of a thoroughly sound and reliable character.

The invention can advantageously be applied in connection with the manufacture of 85 low, medium and high carbon steel rails.

Although the invention has more particularly been described in connection with the manufacture of steel rails, it can, as hereinbefore indicated, advantageously be used in 90 the manufacture of sound steel ingots for conversion into other rolled or forged articles of any desired weight or section. It can also be used in the production of castings of 95 various kinds of sound steel.

What I claim is:—

1. In the manufacture of steel products, the method of ensuring that a normally finished heat of molten steel shall be of a settling nature before casting it into a mould, 100 which consists in transferring a sample of the normally finished steel to a test mould of green sand and allowing it to cool therein and adding to the bath of molten steel, a sufficient quantity of a deoxidizing agent to 105 convert it into steel of a sound and settling nature, if the tested sample shows that the bath of molten steel is of a rising nature, substantially as described.

2. In the manufacture of sound steel ingots, the method of ensuring that a normally finished heat of molten steel shall be of a settling nature before casting it into an ingot mould, which consists in transferring a sample of the normally finished steel to a 110 test mould of green sand and allowing it to cool therein and adding to the bath of molten steel, a sufficient quantity of a deoxidizing agent to convert it into steel of a sound and settling nature, if the tested 115 sample shows that the bath of molten steel is of a rising nature, substantially as described.

Signed at the city of Westminster, London, England, this twenty-fourth day of 125 June, 1926.

ROBERT ABBOTT HADFIELD.